



US005853932A

# United States Patent [19]

Pai et al.

[11] Patent Number: 5,853,932

[45] Date of Patent: Dec. 29, 1998

[54] **LAYERED PHOTORECEPTOR STRUCTURES WITH OVERCOATINGS CONTAINING AN ALKALINE POLYMER**

[75] Inventors: **Damodar M. Pai**, Fairport; **John F. Yanus**, Webster; **Paul J. DeFeo**, Sodus Point; **Dale S. Renfer**, Webster, all of N.Y.

[73] Assignee: **Xerox Corporation**, Stamford, Conn.

[21] Appl. No.: 720,121

[22] Filed: Sep. 27, 1996

[51] Int. Cl.<sup>6</sup> ..... G03G 5/147

[52] U.S. Cl. ..... 430/54; 430/66; 430/126

[58] Field of Search ..... 430/59, 64, 66, 430/67, 126

## [56] References Cited

### U.S. PATENT DOCUMENTS

4,457,994 7/1984 Pai et al. ..... 430/59

4,515,882 5/1985 Mammino et al. ..... 430/58  
5,063,128 11/1991 Yuh et al. ..... 430/63  
5,227,092 7/1993 Hau ..... 252/500  
5,368,967 11/1994 Schank et al. ..... 430/59  
5,384,222 1/1995 Normandin et al. ..... 430/58  
5,384,223 1/1995 Listigovers et al. ..... 430/59  
5,391,447 2/1995 Pai et al. ..... 430/59  
5,401,615 3/1995 Pai et al. ..... 430/59

*Primary Examiner*—John Goodrow

## [57] ABSTRACT

An electrophotographic imaging member including a substrate, a charge generating layer, a charge transport layer including charge transporting molecules dispersed in a polymer binder, and an overcoat layer including an alkaline polymer.

**12 Claims, No Drawings**

**LAYERED PHOTORECEPTOR STRUCTURES  
WITH OVERCOATINGS CONTAINING AN  
ALKALINE POLYMER**

**BACKGROUND OF THE INVENTION**

This invention relates in general to electrophotographic imaging members and more specifically, to layered photoreceptor structures with overcoatings containing alkaline polymers.

Electrophotographic imaging members, i.e. photoreceptors, typically include a photoconductive layer formed on an electrically conductive substrate. The photoconductive layer is a good insulator in the dark so that electric charges are retained on its surface. Upon exposure to light, the charge is dissipated.

A latent image is formed on the photoreceptor by first uniformly depositing an electric charge over the surface of the photoconductive layer by one of any suitable means well known in the art. The photoconductive layer functions as a charge storage capacitor with charge on its free surface and an equal charge of opposite polarity (the counter charge) on the conductive substrate. A light image is then projected onto the photoconductive layer. On those portions of the photoconductive layer that are exposed to light, the electric charge is conducted through the layer reducing the surface charge. The portions of the surface of the photoconductive not exposed to light retain their surface charge. The quantity of electric charge at any particular area of the photoconductive surface is inversely related to the illumination incident thereon, thus forming an electrostatic latent image.

The photodischarge of the photoconductive layer requires that the layer photogenerate conductive charge and transport this charge through the layer thereby neutralizing the charge on the surface. Two types of photoreceptor structures have been employed: multilayer structures wherein separate layers perform the functions of charge generation and charge transport, respectively, and single layer photoconductors which perform both functions. These layers are formed on an electrically conductive substrate and may include an optional charge blocking and an adhesive layer between the conductive layer and the photoconducting layer or layers. Additionally, the substrate may comprise a non-conducting mechanical support with a conductive surface. Other layers for providing special functions such as incoherent reflection of laser light, dot patterns for pictorial imaging or subbing layers to provide chemical sealing and/or a smooth coating surface may be optionally be employed.

One common type of photoreceptor is a multilayered device that comprises a conductive layer, a blocking layer, an adhesive layer, a charge generating layer, and a charge transport layer. The charge transport layer can contain an active aromatic diamine molecule, which enables charge transport, dissolved or molecularly dispersed in a film forming binder. This type of charge transport layer is described, for example in U.S. Pat. No. 4,265,990. Other charge transport molecules disclosed in the prior art include a variety of electron donor, aromatic amines, oxadiazoles, oxazoles, hydrazones and stilbenes for hole transport and electron acceptor molecules for electron transport. Another type of charge transport layer has been developed which utilizes a charge transporting polymer wherein the charge transporting moiety is incorporated in the polymer as a group pendant from the backbone of the polymer backbone or as a moiety in the backbone of the polymer. These types of charge transport polymers include materials such as poly(N-vinylcarbazole), polysilylenes, and others including

those described, for example, in U.S. Pat Nos. 4,618,551, U.S. Pat. No. 4,806,443, U.S. Pat. No. 4,806,444, U.S. Pat. No. 4,818,650, U.S. Pat. Nos. 4,935,487, and 4,956,440. The disclosures of these patents are incorporated herein in their entirety.

Charge generator layers comprise amorphous films of selenium and alloys of selenium and arsenic, tellurium, germanium and the like, hydrogenated amorphous silicon and compounds of silicon and germanium, carbon, oxygen, nitrogen and the like fabricated by vacuum evaporation or deposition. The charge generator layers may also comprise inorganic pigments of crystalline selenium and its alloys; Group II-VI compounds; and organic pigments such as quinacridones, polycyclic pigments such as dibromo anthranthrene pigments, perylene and perinone dianimes, polynuclear aromatic quinones, azo pigments including bis-, tri- and tetrakis-azos; and the like dispersed in a film forming polymeric binder and fabricated by solvent coating techniques.

Phthalocyanines have been employed as photogenerating materials for use in laser printers utilizing infrared exposure systems. Infrared sensitivity is required for photoreceptors exposed to low cost semiconductor laser diode light exposure devices. The absorption spectrum and photosensitivity of the phthalocyanines depend on the central metal atom of the compound. Many metal phthalocyanines have been reported and include, oxyvanadium phthalocyanine, chloro-aluminum phthalocyanine, copper phthalocyanine, oxytitanium phthalocyanine, chlorogallium phthalocyanine, magnesium phthalocyanine and metal-free phthalocyanine. The phthalocyanines exist in many crystal forms which have a strong influence on photogeneration.

One of the design criteria for the selection of the photosensitive pigment for a charge generator layer and the charge transporting molecule for a transport layer is that, when light photons photogenerate holes in the pigment, the holes be efficiently injected into the charge transporting molecule in the transport layer. More specifically, the injection efficiency from the pigment to the transport layer should be high. A second design criterion is that the injected holes be transported across the charge transport layer in a short time; shorter than the time duration between the exposure and development stations in an imaging device. The transit time across the transport layer is determined by the charge carrier mobility in the transport layer. The charge carrier mobility is the velocity per unit field and has dimensions of  $\text{cm}^2/\text{volt sec}$ . The charge carrier mobility is a function of the structure of the charge transporting molecule, the concentration of the charge transporting molecule in the transport layer and the electrically "inactive" binder polymer in which the charge transport molecule is dispersed. It is believed that the injection efficiency can be maximized by choosing a transport molecule whose ionization potential is lower than that of the pigment. However, low ionization potential molecules may have other deficiencies, one of which is their instability in an atmosphere of corona effluents. A copy quality defect resulting from the chemical interaction of the surface of the transport layer with corona effluents is referred to as "parking deletion" and is described in detail below.

Reprographic machines often utilize multilayered organic photoconductors and also employ corotrons or scorotrons to charge the photoconductors prior to imagewise exposure. During the operating lifetime of these photoconductors they are subjected to corona effluents which include ozone, various oxides of nitrogen etc. It is believed that some of these oxides of nitrogen are converted to nitric acid in the presence of water molecules present in the ambient operat-

ing atmosphere. The top surface of the photoconductor is exposed to the nitric acid during operation of the machine and photoconductor molecules at the very top surface of the transport layer are converted to what is believed to be the nitrated species of the molecules and these could form an electrically conductive film. However, during operation of the machine, the cleaning subsystem continuously removes (by wear) a region of the top surface thereby preventing accumulation of the conductive species. However, such is not the case when the machine is not operating (i.e. in idle mode) between two large copy runs. During the idle mode between long copy runs of, for example, 1000 copies, a specific segment of the photoreceptor comes to rest (is parked) beneath a corotron that had been in operation during the long copy run. Although the high voltage to the corotron is turned off during the time period when the photoreceptor is parked, some effluents (e.g. nitric acid, etc.) continue to be emitted from the corotron shield, corotron housing, etc. This effluent emission is concentrated in the region of the stationary photoreceptor parked directly underneath the corotron. The effluents render that surface region electrically conductive. When machine operation is resumed for the next copy run, a loss of resolution, and even deletion, is observed in the affected region. Thus, the corona induced changes primarily occur at the surface region of the charge transport layer. These changes are manifested in the form of increased conductivity which results in loss of resolution of the final toner images. In the case of severe increases in conductivity, there can be regions of severe deletions in the images. The problem of deletion sometimes manifests itself as a loss of resolution when the reprographic machine operates in an extended run of 1000 cycles or more. The onset of loss of resolution depends on the type and number of corotrons employed and the air-flow configuration within the machines. This problem is particularly severe in devices employing the charge transport molecule N,N'-diphenyl-N,N'-bis(3-methylphenyl)-(1,1'-biphenyl)-4,4'-diamine represented by the following structural formula:



Thus, although the charge transport molecule meets most other electrophotographic criteria such as being devoid of traps, having high injection efficiency from many pigments, ease in synthesizing, and inexpensive, it encounters serious parking and other deletion problems when an idle mode is interposed between extended cycling runs.

#### INFORMATION DISCLOSURE STATEMENT

U.S. Pat No. 4,457,994 to Pai et al., issued Jul. 3, 1984—A layered photosensitive member is disclosed comprising a generator layer and a transport layer containing a diamine type molecule dispersed in a polymeric binder and an overcoat containing triphenyl methane molecules dispersed in a polymeric binder.

U.S. Pat. No. 4,515,882 to Mammino et al., issued May 7, 1985—An electrophotographic imaging system is disclosed

which utilizes a member comprising at least one photoconductive layer and an overcoating layer comprising a film forming continuous phase comprising charge transport molecules and finely divided charge injection enabling particles dispersed in the continuous phase, the insulating overcoating layer being substantially transparent to activating radiation to which the photoconductive layer is sensitive and substantially electrically insulating at low electrical fields.

U.S. Pat No. 5,368,967 issued to Schank et al., issued Nov. 29, 1994—An electrophotographic imaging member comprising a substrate, a charge generating layer, a charge transport layer, and an overcoat layer comprising a small molecule hole transporting arylamine having at least two hydroxy functional groups, a hydroxy or multihydroxy triphenyl methane and a polyamide film forming binder capable of forming hydrogen bonds with the hydroxy functional groups of the hydroxy arylamine and hydroxy or multihydroxy triphenyl methane.

U.S. Pat. No. 5,391,447 to Pai et al., issued Feb. 21, 1995—A layered photosensitive member is disclosed comprising a generator layer and a transport layer including charge transporting molecules dispersed in a first polymer binder and an overcoat layer said overcoat including a triphenylmethane molecule dispersed in a second polymer binder.

U.S. Pat. No. 5,401,615 to Pai et al. issued Mar. 28, 1995—An electrophotographic imaging member is disclosed which is fabricated by forming on a charge generating layer a first coating including charge transporting molecules dispersed in a solution of a first polymer binder dissolved in a first solvent, drying the coating to remove the solvent to form a substantially dry charge transport layer, forming on the charge transport layer a second coating including charge transporting molecules and a chemical stabilizer additive selected from the group consisting of a nitrone, isobenzofuran, hydroxyaromatic compound and mixtures thereof molecularly dispersed in an electrically inactive second polymer binder in a solution of a second polymer

binder dissolved in a second solvent, the first polymer binder being insoluble in the second solvent, and drying the second coating to remove the second solvent to form a substantially dry overcoat layer. This electrophotographic imaging member may be utilized in an electrophotographic imaging process.

U.S. Pat. No. 5,384,222 issued to Normandin et al. on Jan. 24, 1995—A process is disclosed for preparation of a photogenerating composition comprising mixing titanyl phthalocyanine Type IV with the AB block copolymer polystyrene-4-vinyl pyridine.

U.S. Pat. No. 5,384,223 issued to Listigovers et al. on Jan. 24, 1996—A photoconductive imaging member is disclosed comprising a supporting substrate, a photogenerating layer comprising photogenerating pigments dispersed in a polystyrene/polyvinyl pyridine ( $A_n-B_m$ ) block copolymer

wherein n represents the degree of polymerization of A and m represents the degree of polymerization of B, and a charge transport layer.

Although the inventions of the prior art meet the criteria for increased deletion resistance, the overcoat of the prior art contain several materials. There is a need for a simple single component overcoat that improves the deletion resistance without introducing cyclic instabilities.

Thus, there is a continuing need for photoreceptors having improved resistance to increased densities in the background areas of the final images, resistance to migration of additives into the generator layer during fabrication of the transport layer, and resistance to cyclic instabilities.

#### SUMMARY OF THE INVENTION

It is, therefore, an object of the present invention to provide an improved electrophotographic imaging member which overcomes the above-noted deficiencies.

It is yet another object of the present invention to provide an improved electrophotographic imaging member capable of reproducing extremely high resolution images.

It is still another object of the present invention to provide an improved electrophotographic imaging member having a surface region stable against loss of resolution.

It is another object of the present invention to provide an improved electrophotographic imaging member having a surface region stable against copy defects such as print deletion.

It is yet another object of the present invention to provide an improved electrophotographic imaging member having greater stability against corona effluents without an attendant reduction in transport efficiency of transport layers.

It is still another object of the present invention to provide an improved electrophotographic imaging member having greater stability against corona effluents without an attendant reduction of the sensitivity of the imaging member.

The foregoing objects and others are accomplished in accordance with this invention by providing an electrophotographic imaging member comprising a substrate, a charge generating layer, a charge transport layer comprising charge transporting molecules dispersed in a polymer binder, and an overcoat layer comprising an alkaline polymer. The expression alkaline polymer, as employed, is defined as a "basic polymer". The term "basic" is intended to refer to Lewis type basicity which is defined as a chemical moiety able to donate a pair of electrons. Organic species containing nitrogen are examples of such basic moieties, as evidenced by their basic ionization constants, for example, trimethylamine  $K_b=5.5\times 10^{-4}$ , aniline  $K_b=4.2\times 10^{-10}$ , pyridine  $K_b=2.3\times 10^{-9}$ . Typical basic or alkaline polymer structures are represented by the formula:



wherein:

n represents the degree of polymerization and is a number between about 2 and about 50,

m represents the degree of polymerization and can be a number between 50 and 1500,

Y is selected from the group consisting of:



5 X is selected from the group consisting of  
10  $-\text{CHCH}_3\text{COOCH}_3$ ,  $-\text{CH}_2\text{COOCH}_3$  and



$R_1, R_2, R_3, R_4, R_5$  and  $R_6$  are independently selected from the group consisting of  $\text{H}, -\text{CH}_3, -\text{CH}_2\text{CH}_3, -\text{CH}_2\text{CH}(\text{CH}_3)_2$  and  $-\text{CH}_2\text{C}(\text{CH}_3)_3$ , and  
20  $R_7$  and  $R_8$  are independently selected from  $\text{H}, -\text{CH}_3, -\text{CH}_2\text{CH}_3, -\text{CH}_2\text{CH}(\text{CH}_3)_2, -\text{CH}_2\text{C}(\text{CH}_3)_3$ , and  
25  $-\text{OR}_9$  wherein  $R_9$  is defined as  $R_1 - R_6$  above.

25 The photoreceptor device of this invention may also include any suitable optional charge blocking, adhesive and other sub layers. This electrophotographic imaging member is fabricated by forming on a charge generating layer, a transport layer comprising charge transporting molecules dissolved or molecularly dispersed in a film forming polymer binder, forming on the charge transport layer an overcoat of an alkaline film forming polymer containing charge transporting small molecules. This electrophotographic imaging member may be utilized in an electrophotographic imaging process.

30 35 Electrophotographic imaging members are well known in the art. Electrophotographic imaging members may be prepared by any suitable technique. Typically, a flexible or rigid substrate is provided with an electrically conductive surface. A charge generating layer is then applied to the electrically 40 conductive surface. A charge blocking layer may optionally be applied to the electrically conductive surface prior to the application of a charge generating layer. If desired, an adhesive layer may be utilized between the charge blocking layer and the charge generating layer. Usually the charge 45 generation layer is applied onto the blocking layer and a charge transport layer is formed on the charge generation layer. This structure may have the charge generation layer on top of or below the charge transport layer.

50 The substrate may be opaque or substantially transparent and may comprise any suitable material having the required mechanical properties. Accordingly, the substrate may comprise a layer of an electrically non-conductive or conductive material such as an inorganic or an organic composition. As electrically non-conducting materials there may be

55 employed various resins known for this purpose including polyesters, polycarbonates, polyamides, polyurethanes, and the like which are flexible as thin webs. An electrically conducting substrate may be any metal, for example, aluminum, nickel, steel, copper, and the like or a polymeric

60 material, as described above, filled with an electrically conducting substance, such as carbon, metallic powder, and the like or an organic electrically conducting material. The electrically insulating or conductive substrate may be in the form of an endless flexible belt, a web, a rigid cylinder, a sheet and the like.

65 The thickness of the substrate layer depends on numerous factors, including strength desired and economical consid-

erations. Thus, for a drum, this layer may be of substantial thickness of, for example, up to many centimeters or of a minimum thickness of less than a millimeter. Similarly, a flexible belt may be of substantial thickness, for example, about 250 micrometers, or of minimum thickness less than 50 micrometers, provided there are no adverse effects on the final electrophotographic device.

In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors. Accordingly, for a flexible photoresponsive imaging device, the thickness of the conductive coating may be between about 20 angstroms to about 750 angstroms, and more preferably from about 100 angstroms to about 200 angstroms for an optimum combination of electrical conductivity, flexibility and light transmission. The flexible conductive coating may be an electrically conductive metal layer formed, for example, on the substrate by any suitable coating technique, such as a vacuum depositing technique or electrodeposition. Typical metals include aluminum, zirconium, niobium, tantalum, vanadium and hafnium, titanium, nickel, stainless steel, chromium, tungsten, molybdenum, and the like.

An optional hole blocking layer may be applied to the substrate. Any suitable and conventional blocking layer capable of forming an electronic barrier to holes between the adjacent photoconductive layer and the underlying conductive surface of a substrate may be utilized.

An optional adhesive layer may be applied to the hole blocking layer. Any suitable adhesive layer well known in the art may be utilized. Typical adhesive layer materials include, for example, polyesters, polyurethanes, and the like. Satisfactory results may be achieved with adhesive layer thickness between about 0.05 micrometer (500 angstroms) and about 0.3 micrometer (3,000 angstroms). Conventional techniques for applying an adhesive layer coating mixture to the charge blocking layer include spraying, dip coating, roll coating, wire wound rod coating, gravure coating, Bird applicator coating, and the like. Drying of the deposited coating may be effected by any suitable conventional technique such as oven drying, infra red radiation drying, air drying and the like.

Any suitable polymeric film forming binder material may be employed as the matrix in the charge generating (photogenerating) binder layer. Typical polymeric film forming materials include those described, for example, in U.S. Pat No. 3,121,006, the entire disclosure of which is incorporated herein by reference. Thus, typical organic polymeric film forming binders include thermoplastic and thermosetting resins such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl acetate, polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, polyvinylchloride, vinylchloride and vinyl acetate copolymers, acrylate copolymers, alkyd resins, cel-

lulosic film formers, poly(amideimide), styrene-butadiene copolymers, vinylidenechloride-vinylchloride copolymers, vinylacetate-vinylidenechloride copolymers, styrene-alkyd resins, polyvinylcarbazole, and the like. These polymers may be block, random or alternating copolymers.

The photogenerating composition or pigment is present in the resinous binder composition in various amounts. Generally, however, from about 5 percent by volume to about 90 percent by volume of the photogenerating pigment is dispersed in about 10 percent by volume to about 95 percent by volume of the resinous binder, and preferably from about 20 percent by volume to about 30 percent by volume of the photogenerating pigment is dispersed in about 15 percent by volume to about 80 percent by volume of the resinous binder composition. In one embodiment about 8 percent by volume of the photogenerating pigment is dispersed in about 92 percent by volume of the resinous binder composition. The photogenerator layers can also be fabricated by vacuum sublimation in which case there is no binder.

Any suitable and conventional technique may be utilized to mix and thereafter apply the photogenerating layer coating mixture. Typical application techniques include 25 spraying, dip coating, roll coating, wire wound rod coating, vacuum sublimation and the like. For some applications, the generator layer may be fabricated in a dot or line pattern. Removing of the solvent of a solvent coated layer may be effected by any suitable conventional technique such as oven 30 drying, infrared radiation drying, air drying and the like.

The charge transport layer may comprise a charge transporting small molecule dissolved or molecularly dispersed in a film forming electrically inert polymer such as a polycarbonate. The term "dissolved" as employed herein is 35 defined herein as forming a solution in which the small molecule is dissolved in the polymer to form a homogeneous phase. The expression "molecularly dispersed" is used herein as defined as a charge transporting small molecule dispersed in the polymer, the small molecules being dispersed in the polymer on a molecular scale. Any suitable charge transporting or electrically active small molecule 40 may be employed in the charge transport layer of this invention. The expression charge transporting "small molecule" is defined herein as a monomer that allows the free charge photogenerated in the transport layer to be transported across the transport layer. Typical charge transporting small molecules include, for example, pyrazolines such as 45 1-phenyl-3-(4'-diethylamino styryl)-5-(4"-diethylamino phenyl)pyrazoline, diamines such as N,N'-diphenyl-N,N'-bis(3-methylphenyl)-(1,1'-biphenyl)-4,4'-diamine, hydrazones such as N-phenyl-N-methyl-3-(9-ethyl)carbazyl 50 hydrazone and 4-diethyl amino benzaldehyde-1,2-diphenyl hydrazone, and oxadiazoles such as 2,5-bis(4-N,N'-diethylaminophenyl)-1,2,4-oxadiazole, stilbenes and the like. However, to avoid cycle-up, the charge transport layer 55 should be substantially free of triphenyl methane. As indicated above, suitable electrically active small molecule charge transporting compounds are dissolved or molecularly dispersed in electrically inactive polymeric film forming materials. A small molecule charge transporting compound 60 that permits injection of holes from the pigment into the charge generating layer with high efficiency and transports them across the charge transport layer with very short transit times is N,N'-diphenyl-N,N'-bis(3-methylphenyl)-(1,1'-biphenyl)-4,4'-di-amine represented by the formula:



The electrically inert polymeric binder generally used to disperse the electrically active molecule in the charge transport layer is a poly(4,4'-isopropylidene-diphenylene) carbonate (also referred to as bisphenol-A-polycarbonate) represented by the formula:



Any suitable electrically inactive resin binder insoluble in the solvent used to apply the overcoat layer may be employed in the charge transport layer of this invention. Typical inactive resin binders include polycarbonate resin, polyester, polyarylate, polyacrylate, polyether, polysulfone, and the like. Molecular weights can vary, for example, from about 20,000 to about 150,000.

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like.

Generally, the thickness of the charge transport layer is between about 10 and about 50 micrometers, but thicknesses outside this range can also be used. The hole transport layer should be an insulator to the extent that the electrostatic charge placed on the hole transport layer is not conducted in the absence of illumination at a rate sufficient to prevent formation and retention of an electrostatic latent image thereon. In general, the ratio of the thickness of the hole transport layer to the charge generator layers is preferably maintained from about 2:1 to 200:1 and in some instances as great as 400:1. In other words, the charge transport layer, is substantially non-absorbing to visible light or radiation in the region of intended use but is electrically "active" in that it allows the injection of photogenerated holes from the photoconductive layer, i.e., charge generation layer, and allows these holes to be transported through itself to selectively discharge a surface charge on the surface of the active layer.

The overcoat layer of this invention comprises any suitable alkaline (basic) polymer having Lewis type basicity, defined as a chemical moiety able to donate a pair of electrons. Polymers conforming to this definition are represented by the following  $(A_n-B_m)$  block co-polymer formula:



wherein:

n represents the degree of polymerization and is a number between about 2 and about 50,

m represents the degree of polymerization and is a number between 50 and 1500,

Y is selected from the group consisting of:



X is selected from the group consisting of  $-CH_2CH_3COOCH_3$ ,  $-CH_2COOCH_3$  and



R<sub>1</sub>, R<sub>2</sub>, R<sub>3</sub>, R<sub>4</sub>, R<sub>5</sub> and R<sub>6</sub> are independently selected from H,  $-CH_3$ ,  $-CH_2CH_3$ ,  $-CH_2CH(CH_3)_2$ , and  $-CH_2C(CH_3)_3$ , and

R<sub>7</sub> and R<sub>8</sub> are independently selected from H,  $-CH_3$ ,  $-CH_2CH_3$ ,  $-CH_2CH(CH_3)_2$ ,  $-CH_2C(CH_3)_3$  and  $-OR_9$  wherein R<sub>9</sub> is defined as R<sub>1</sub>—R<sub>6</sub> above.

A preferred alkaline polymer is a polystyrene/polyvinyl pyridine block copolymer wherein n can be, for example, a number between about 7 and about 50, such as 4-vinyl pyridine, and wherein m can be, for example, a number between about 70 and about 800 such as styrene, with compositional ratios of the 4-vinyl-pyridine to styrene in the range of between about 5/95 and about 30/70 and more preferably in the range between about 8/92 and about 20/80.—Examples of pyridine moieties for the copolymers include poly(2-vinylpyridine) and poly(4-vinylpyridine). Examples of polystyrene moieties include polystyrene and poly[p-(dimethylamino methyl)styrene]. Polystyrene/polyvinyl pyridine (A<sub>n</sub>-B<sub>m</sub>) block copolymers and processes for synthesizing them are described in U.S. Pat. No. 5,384,222 and U.S. Pat. No. 5,384,223, the disclosures of these two patents are incorporated herein by reference in

their entirety. Other typical alkaline (basic) polymers having Lewis type basicity include for example, polyvinyl-4-pyridine-co-polymethacrylate, poly-4-dimethylaminostyrene-co-polystyrene, poly-4-dimethylaminostyrene-co-poly(methylmethacrylate), and the like. The above polystyrene/polyvinyl pyridine block copolymer formula includes copolymers of polystyrene and polyvinyl pyridines such as polystyrene/poly-4-vinyl pyridine with, for example, a  $M_w$  of between about 7,000 and about 80,000 and more preferably between about 10,500 and about 40,000, and a  $M_n$  of between about 5,500 and about 60,200, and preferably between about 8,000 and about 22,800, and wherein the percentage of vinyl pyridine is between about 5 and about 55 and preferably between about 9 and about 20. The remaining percentage being made up of a polystyrene block.

The block copolymers can be synthesized by anionic polymerization, reference the processes as illustrated in K. Ishizu, Y. Kashi, T. Fujutomi, T. Kakurai, *Makromol. Chem.* 183, pages 3090 to 3107 (1982), the disclosure of which is incorporated herein by reference in its entirety. For example, anionic polymerization of styrene-b-4-vinylpyridine can be accomplished at a temperature of from about -10° C. to about -50° C. in solvents such as tetrahydrofuran (THF) by initiation of styrene monomer with the  $\alpha$ -methylstyryl anion generated from  $\alpha$ -methylstyrene and a component like such as n-butyllithium (n-BuLi). Reaction is essentially instantaneous to yield the polystyrene stabilizing block with molecular weights which are easily calculated from the ratio of the total weight of monomer to the number of moles of initiator, and are as indicated herein. The living polystyryl anions are then further reacted with 4-vinylpyridine monomer to provide the desired anchoring block with little or no increase in polydispersity. The reaction is quenched with methanol and precipitated directly into deionized water. After filtering and vacuum drying, the block copolymer is obtained as a white powder in 96 percent yield. One typical styrene/4-vinylpyridine block copolymer contains 10 weight percent of 4-vinylpyridine and 90 weight percent of styrene, as determined by  $^1\text{H}$  NMR, and has a weight average molecular of 15,000 as determined by GPC. Copolymers with narrow polydispersities, such as for example a molecular weight distribution ( $M_w/M_n$ ) of less than about 1.2, can be selected. Composition and molecular weight of the copolymers can be controlled and determined by the weight of monomers used in the reaction and the stoichiometric ratio of the  $\alpha$ -methylstyryl anion to the styrene and 4-vinylpyridine monomers. For example, if 90 grams of styrene are polymerized followed with 10 grams of 4-vinylpyridine, the final copolymer will contain 10 weight percent of 4-vinylpyridine. When 1 millimol of initiator is used to polymerize the 100 grams of monomer, then the molecular weight measured by GPC will be in the range of 100,000.

The thickness of the overcoat layer selected depends upon the abrasiveness of the cleaning system employed and can range from about 0.5 micrometer to about 10 micrometers in thickness. Any suitable and conventional technique may be utilized to mix and thereafter apply the overcoat layer coating mixture to the charge generating layer. Typical application techniques include spraying, dip coating, roll coating, wire wound rod coating, and the like. Drying of the deposited coating may be effected by any suitable conventional technique such as oven drying, infrared radiation drying, air drying and the like.

During the coating step for application of the overcoat onto the charge transport layer, the charge transporting small

molecules from the transport layer may migrate into the overcoat layer and impart to the overcoat the charge transporting property. If desired, the overcoat alkaline polymer may optionally be predoped with the charge transporting small molecules prior to the overcoat application coating step and not rely on migration of the charge transport molecules from the charge transport layer during the overcoat application step. Whether the final overcoat contains migrated charge transporting small molecules from the transport layer and/or predoped charge transporting small molecules, the total amount of charge transport molecules dissolved or molecularly dispersed in the alkaline polymer of the final dried overcoat is preferably between about 5 and about 30 weight percent, based on the total weight of the dried overcoating layer. The overcoating may contain any suitable charge transporting molecules dissolved or molecularly dispersed in the alkaline polymer. As described above, the expression charge transporting "small molecule" is defined herein as a monomer that allows the free charge photogenerated in the transport layer to be transported across the transport layer. Typical charge transporting small molecules include, for example, pyrazolines such as 1-phenyl-3-(4'-diethylamino styryl)-5-(4"-diethylamino phenyl)pyrazoline, diamines such as N,N'-bis(3-methylphenyl)-(1,1'-biphenyl)-4,4'-diamine, hydrazones such as N-phenyl-N-methyl-3-(9-ethyl)carbazyl hydrazone and 4-diethyl amino benzaldehyde-1,2-diphenyl hydrazone, and oxadiazoles such as 2,5-bis (4-N,N'-diethylaminophenyl)-1,2,4-oxadiazole, stilbenes and the like.

Other suitable layers may also be used such as a conventional electrically conductive ground strip along one edge of the belt or drum in contact with the conductive surface of the substrate to facilitate connection of the electrically conductive layer of the photoreceptor to ground or to an electrical bias. Ground strips are well known and usually comprise conductive particles dispersed in a film forming binder.

In some cases an anti-curl back coating may be applied to the side opposite the photoreceptor to provide flatness and/or abrasion resistance for belt or web type photoreceptors. These anti-curl back coating layers are well known in the art and may comprise thermoplastic organic polymers or inorganic polymers that are electrically insulating or slightly semiconducting.

The photoreceptor of this invention may be used in any conventional electrophotographic imaging system. As described above, electrophotographic imaging usually involves depositing a uniform electrostatic charge on the photoreceptor, exposing the photoreceptor to a light image pattern to form an electrostatic latent image on the photoreceptor, developing the electrostatic latent image with electrostatically attractive marking particles to form a visible toner image, transferring the toner image to a receiving member and repeating the depositing, exposing, developing and transferring steps at least once. The serious parking and other deletion problems when an idle mode is interposed between extended cycling runs become especially pronounced when the depositing, exposing, developing and transferring steps are repeated at least 1,000 times in a single run, followed by resting of the photoreceptor between about 5 minutes and about 30 minutes, and repeating said depositing, exposing, developing and transferring steps at least 10 additional times in another single run.

A number of examples are set forth hereinbelow and are illustrative of different compositions and conditions that can be utilized in practicing the invention. All proportions are by weight unless otherwise indicated. It will be apparent,

## 13

however, that the invention can be practiced with many types of compositions and can have many different uses in accordance with the disclosure above and as pointed out hereinafter.

## EXAMPLE I

Two photoreceptors are prepared by forming coatings using conventional techniques on a substrate comprising a vacuum deposited titanium layer on a polyethylene terephthalate film. The first coating is a siloxane barrier layer formed from hydrolyzed gamma aminopropyltriethoxysilane having a thickness of 0.005 micrometer (50 Angstroms). The barrier layer coating composition is prepared by mixing 3-aminopropyltriethoxysilane (available from PCR Research Chemicals of Florida) with ethanol in a 1:50 volume ratio. The coating composition is applied by a multiple clearance film applicator to form a coating having a wet thickness of 0.5 mil. The coating is then allowed to dry for 5 minutes at room temperature, followed by curing for 10 minutes at 110 degrees centigrade in a forced air oven. The second coating is an adhesive layer of polyester resin (49,000, available from E. I. duPont de Nemours & Co.) having a thickness of 0.005 micron (50 Angstroms). The second coating composition is prepared by dissolving 0.5 gram of 49,000 polyester resin in 70 grams of tetrahydrofuran and 29.5 grams of cyclohexanone. The second coating composition is applied using a 0.5 mil bar and the resulting coating is cured in a forced air oven for 10 minutes. The next coating is a charge generator layer containing 35 percent by weight vanadyl phthalocyanine particles obtained by the process as disclosed in U.S. Pat. No. 4,771,133, dispersed in a polyester resin (Vitel PE100, available from Goodyear Tire and Rubber Co.) having a thickness of 1 micrometer. The next layer is a charge transport layer and is coated with a solution containing one gram of N,N'-diphenyl-N,N'-bis(3-methyl-phenyl)-(1,1'biphenyl)-4,4'-diamine and one gram of polycarbonate resin [poly(4,4'-isopropylidene-diphenylene carbonate, available as Makrolon® from Farbenfabriken Bayer A. G.], dissolved in 11.5 grams of methylene chloride solvent using a Bird coating applicator. The N,N'-diphenyl-N,N'-bis(3-methyl-phenyl)-(1,1'biphenyl)-4,4'-diamine is an electrically active aromatic diamine charge transport small molecule whereas the polycarbonate resin is an electrically inactive film forming binder. The coated device is dried at 80° C. for half an hour in a forced air oven to form a 25 micrometer thick charge transport layer.

## EXAMPLE II

One of two photoconductors fabricated as described in Example I is overcoated with a block copolymer of styrene (82 percent)/4-vinyl Pyridine (18 percent) having a Mw of 11,900. 0.5 gram of this polymer is dissolved in 7 grams of methylene chloride and an overcoat film is coated with a bar containing 0.5 mil bar. The resulting device is heated at 100° C. for 30 minutes. The overcoat thickness is 3 micrometers.

## EXAMPLE III

Deletion resistance test: A negative corotron is operated (with high voltage connected to the corotron wire) opposite a grounded electrode for several hours. The high voltage is turned off, and the corotron is placed (or parked) for thirty minutes on a segment of the photoconductor device being tested. Only a short middle segment of the device is thus exposed to the corotron effluents. Unexposed regions on either side of the exposed regions are used as controls. The

## 14

photoconductor device is then tested in a scanner for positive charging properties for systems employing donor type molecules. These systems are operated with negative polarity corotron in the latent image formation step. An electrically conductive surface region (excess hole concentration) appears as a loss of positive charge acceptance or increased dark decay in the exposed regions (compared to the unexposed control areas on either side of the short middle segment) Since the electrically conductive region is located on the surface of the photoreceptor device, a negative charge acceptance scan is not affected by the corotron effluent exposure (negative charges do not move through a charge transport layer made up of donor molecules). However, the excess carriers on the surface cause surface conductivity resulting in loss of image resolution and, in severe cases, causes deletion. The photoreceptor devices of Example I (without the overcoat of this invention) and Example II (with the overcoat of this invention) are tested for deletion resistance. The region not exposed to corona effluents charged to 1000 positive in both devices; however the corona exposed region of device of Example I is charged to 500 volts (a loss of 500 volts of charge acceptance) whereas the corona exposed region of device of Example II is charged to 800 volts (a loss of 200 volts of charge acceptance). The overcoat has improved the deletion resistance by a factor of 2.5.

## EXAMPLE IV

Both photoreceptor devices of Example I and II are mounted on a cylindrical aluminum drum substrate which is rotated on a shaft. The device is charged by a corotron mounted along the periphery of the drum. The surface potential is measured as a function of time by capacitively coupled voltage probes placed at different locations around the shaft. The probes are calibrated by applying known potentials to the drum substrate. The devices on the drums are exposed by a light source located at a position near the drum downstream from the corotron. As the drum is rotated, the initial (pre exposure) charging potential is measured by voltage probe 1. Further rotation leads to the exposure station, where the photoreceptor device is exposed to monochromatic radiation of known intensity. The device is erased by light source located at a position upstream of charging. The measurements made include charging of the photoconductor device in a constant current or voltage mode. The device is charged to a negative polarity corona. As the drum is rotated, the initial charging potential is measured by voltage probe 1. Further rotation leads to the exposure station, where the photoconductor device is exposed to monochromatic radiation of known intensity. The surface potential after exposure is measured by voltage probes 2 and 3. The device is finally exposed to an erase lamp of appropriate intensity and any residual potential is measured by voltage probe 4. The process is repeated with the magnitude of the exposure automatically changed during the next cycle. The photodischarge characteristics is obtained by plotting the potentials at voltage probes 2 and 3 as a function of light exposure. The charge acceptance and dark decay can also be measured in the scanner. The sensitivity of the overcoated device is slightly higher as a result of the increased total thickness. The cyclic stability of the overcoated device is equal to that of the unovercoated device. There is no residual cycle-up as a result of the overcoat.

## EXAMPLE V

Two photoreceptors are prepared as described in Example I until the blocking interface and adhesive layers are coated.

## 15

The adhesive interface layer is thereafter coated with a photogenerating layer containing 40 percent by volume hydroxygallium phthalocyanine and 60 percent by volume of a block copolymer of styrene (82 percent)/4-vinyl pyridine (18 percent) having a  $M_w$  of 11,900. This photogenerating coating composition is prepared by dissolving 1.5 grams of the block copolymer of styrene/4-vinyl pyridine in 42 ml of toluene. To this solution is added 1.33 grams of hydroxygallium phthalocyanine and 300 grams of  $\frac{1}{8}$  inch diameter stainless steel shot. This mixture is then placed on a ball mill for 20 hours. The resulting slurry is thereafter applied to the adhesive interface with a Bird applicator to form a layer having a wet thickness of 0.25 mil.

This layer is dried at 135° C. for 5 minutes in a forced air oven to form a photogenerating layer having a dry thickness 15 0.4 micrometer. The next applied layer is a transport layer which is formed by using a Bird coating applicator to apply a solution containing one gram of N,N'-diphenyl-N,N'-bis(3-methyl-phenyl)-(1,1'biphenyl)-4,4'-diamine and one gram of polycarbonate resin [poly(4,4'-isopropylidene-diphenylene carbonate (available as Makrolon® from Farbenfabriken Bayer A. G.) dissolved in 11.5 grams of methylene chloride solvent. The N,N'-diphenyl-N,N'-bis(3-methyl-phenyl)-(1,1'biphenyl)-4,4'-diamine is an electrically active aromatic diamine charge transport small molecule whereas the polycarbonate resin is an electrically inactive film forming binder. The coated device is dried at 20 80° C. for half an hour in a forced air oven to form a dry 25 25 0.25 micrometer thick charge transport layer.

## EXAMPLE VI

The second photoreceptor of Example V is overcoated with with a block copolymer of styrene (82 percent)/4-vinyl Pyridine (18 percent) having a  $M_w$  of 11,900. 0.5 gram of this polymer is dissolved in 7 gms of methylene chloride and an overcoat film was coated with a bar containing 0.5 mil bar. The resulting photoreceptor device is heated at 100° C. for 30 minutes. The overcoat thickness is 3 micrometers.

## EXAMPLE VII

The photoreceptor devices of Examples V and VI are tested for deletion resistance as described in Example III. The overcoated photoreceptor device of Example VI has a deletion resistance 3 times superior to the unovercoated photoreceptor device of Example V.

## EXAMPLE VIII

The photoreceptor devices of Examples V and VI are tested for their sensitivity and cyclic stability in a scanner as described in Example IV. The overcoated photoreceptor device of Example VI has a slightly higher sensitivity as a result of the increased thickness. The cyclic stability of the overcoated photoreceptor device is equal to that of the unovercoated photoreceptor device. There is no residual cycle-up as a result of the overcoat.

Although the invention has been described with reference to specific preferred embodiments, it is not intended to be limited thereto, rather those skilled in the art will recognize that variations and modifications may be made therein which are within the spirit of the invention and within the scope of the claims.

What is claimed is:

1. An electrophotographic imaging member comprising a substrate, a charge generating layer, a charge transport layer and an overcoat layer comprising an alkaline polymer.
2. An electrophotographic imaging member according to claim 1 wherein said alkaline polymer is represented by the following ( $A_n-B_m$ ) block co-polymer formula:

5

## 16



wherein:

n represents the degree of polymerization and can be a number between about 2 and about 50,

m represents the degree of polymerization and is a number between 50 and 1500,

Y is selected from the group consisting of:



X is selected from the group consisting of —CHCH3COOCH3, —CH2COOCH3 and



R1, R2, R3, R4, R5 and R6 are independently selected from the group consisting of H, —CH3, —CH2CH3, —CH2CH(CH3)2, and —CH2C(CH3)3,

R7 and R8 are independently selected from the group consisting of H, —CH3, —CH2CH3, —CH2CH(CH3)2, —CH2C(CH3)3 and —OR9 where R9 is defined as R1—R6 above.

3. An electrophotographic imaging member according to claim 1 wherein said alkaline polymer is a polystyrene/polyvinyl pyridine ( $A_n-B_m$ ) block copolymer wherein n represents the degree of polymerization of A and m represents the degree of polymerization of B and said block copolymer has a weight average weight between about 7,000 and about 80,000.

4. An electrophotographic imaging member according to claim 1 wherein said charge transport layer comprises electrically active charge transporting molecules dissolved or 40 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380

of a blocking layer, adhesive layer and combination thereof are interposed between said substrate and said charge generating layer.

**10.** An electrophotographic imaging member according to claim **1** wherein said charge transport layer has a thickness of between about 5 micrometers and about 50 micrometers.

**11.** An imaging process comprising providing an electrophotographic imaging member comprising a charge generating layer, a charge transport layer and an overcoat layer comprising an alkaline polymer, exposing said imaging member to a light image pattern to form an electrostatic latent image on said imaging member, developing said electrostatic latent image with electrostatically attractable

toner particles to form a visible toner image, transferring said toner image to a receiving member and repeating said depositing, exposing, developing and transferring steps at least once.

**12.** An imaging process according to claim **11** including repeating said depositing, exposing, developing and transferring steps at least 1,000 times in a single run, resting said imaging member between about 5 minutes and about 30 minutes, and repeating said depositing, exposing, developing and transferring steps at least 10 additional times in another single run.

\* \* \* \* \*